



US005080814A

# United States Patent [19]

Awad

[11] Patent Number: 5,080,814

[45] Date of Patent: \* Jan. 14, 1992

[54] AQUEOUS LUBRICANT AND SURFACE CONDITIONER FOR FORMED METAL SURFACES

[75] Inventor: Sami B. Awad, Troy, Mich.

[73] Assignee: Henkel Corporation, Ambler, Pa.

[\*] Notice: The portion of the term of this patent subsequent to Aug. 22, 2006 has been disclaimed.

[21] Appl. No.: 521,219

[22] Filed: May 8, 1990

## Related U.S. Application Data

[63] Continuation of Ser. No. 395,620, Aug. 18, 1989, Pat. No. 4,944,889, which is a continuation-in-part of Ser. No. 57,129, Jun. 1, 1987, Pat. No. 4,859,351.

[51] Int. Cl.<sup>5</sup> ..... C10M 173/00; B65D 75/00

[52] U.S. Cl. ..... 252/49.3; 252/41; 252/49.8; 252/51.5 A; 252/52 A; 252/56 R; 206/139

[58] Field of Search ..... 252/41, 49.3, 49.8, 252/51.5 A, 52 A, 56 R; 206/139

## References Cited

### U.S. PATENT DOCUMENTS

|           |         |                 |       |          |
|-----------|---------|-----------------|-------|----------|
| 2,285,853 | 6/1942  | Downing et al.  | ..... | 252/53   |
| 3,860,521 | 1/1975  | Aepli et al.    | ..... | 252/34.7 |
| 3,923,471 | 12/1975 | Smith et al.    | ..... | 29/195   |
| 3,945,930 | 3/1976  | Sugiyama et al. | ..... | 252/52 A |
| 4,116,872 | 9/1978  | Jahnke          | ..... | 252/32.7 |
| 4,212,750 | 7/1980  | Gorman          | ..... | 252/32.5 |
| 4,215,002 | 7/1980  | Fein            | ..... | 252/32.5 |
| 4,260,499 | 4/1981  | Fein et al.     | ..... | 252/32.5 |
| 4,521,321 | 6/1985  | Anderson et al. | ..... | 252/49.3 |

|           |         |                     |       |          |
|-----------|---------|---------------------|-------|----------|
| 4,601,838 | 7/1986  | Kammann, Jr. et al. | ..... | 252/49.3 |
| 4,604,220 | 8/1986  | Stanton             | ..... | 252/33.4 |
| 4,612,128 | 9/1986  | Uematsu et al.      | ..... | 252/32.5 |
| 4,637,885 | 1/1987  | Kuwamoto et al.     | ..... | 252/32.5 |
| 4,650,595 | 3/1987  | Nagamori et al.     | ..... | 252/32.5 |
| 4,657,685 | 4/1987  | Uematsu et al.      | ..... | 252/32.5 |
| 4,710,409 | 12/1987 | Lahaye              | ..... | 427/421  |
| 4,731,190 | 3/1988  | O'Lenick et al.     | ..... | 252/49.3 |
| 4,752,405 | 6/1988  | Kyle et al.         | ..... | 252/41   |
| 4,758,359 | 7/1988  | Kirk et al.         | ..... | 252/49.3 |
| 4,859,351 | 8/1989  | Awad                | ..... | 252/32.5 |
| 4,944,889 | 7/1990  | Awad                | ..... | 252/32.5 |
| 4,950,415 | 8/1990  | Malito              | ..... | 252/49.3 |

## OTHER PUBLICATIONS

GAF Corporation, Wayne, N.J.—pp. 1-51.  
Ethox Chemicals, Inc., Greenville, S.C.—pp. 1-16.

Primary Examiner—Prince Willis, Jr.

Assistant Examiner—Jerry D. Johnson

Attorney, Agent, or Firm—Ernest G. Szoke; Wayne C. Jaeschke; Norvell E. Wisdom, Jr.

## ABSTRACT

A lubricant and surface conditioner for formed metal surfaces, particularly beverage containers, which reduces the coefficient of static friction of said metal surfaces and enables drying said metal surfaces at a lower temperature.

The conditioner is a water-soluble organic material selected from a phosphate ester, alcohol, fatty acid including mono-, di-, tri-, and poly-acids; fatty acid derivatives such as salts, hydroxy acids, amides, esters, ethers and derivatives thereof; and mixtures thereof.

20 Claims, No Drawings

## AQUEOUS LUBRICANT AND SURFACE CONDITIONER FOR FORMED METAL SURFACES

## BACKGROUND OF THE INVENTION

## 1. Field of the Invention

This application is a continuation of copending application Ser. No. 395,620 filed Aug. 18, 1989, now U.S. Pat. No. 4,944,889 which was a continuation-in-part of Ser. No. 057,129 filed June 1, 1987 now U.S. Pat. No. 4,859,351. 10

This invention relates to a lubricant and surface conditioner for formed metal surfaces, and more particularly, to such a lubricant and surface conditioner which improves the mobility of aluminum cans without adversely affecting the adhesion of paints or lacquers applied thereto, and also enables lowering the dryoff oven temperature required for drying said surfaces.

## 2. Discussion of Related Art

2. Discussion of Related API

Aluminum cans are commonly used as containers for a wide variety of products. After their manufacture, the aluminum cans are typically washed with acidic cleaners to remove aluminum fines and other contaminants therefrom. Recently, environmental considerations and the possibility that residues remaining on the cans following acidic cleaning could influence the flavor of beverages packaged in the cans has led to an interest in alkaline cleaning to remove such fines and contaminants. However, the treatment of aluminum cans generally results in differential rates of metal surface etch on the outside versus on the inside of the cans. For example, optimum conditions required to attain an aluminum fine-free surface on the inside of the cans usually leads to can mobility problems on conveyors because of the increased roughness on the outside can surface.

These aluminum can mobility problems are particularly apparent when it is attempted to convey the cans through single filers and to printers. Thus, a need has arisen in the aluminum can manufacturing industry to 40 modify the coefficient of static friction on the outside surface of the cans to improve their mobility without adversely affecting the adhesion of paints or lacquers applied thereto. The reason for improving the mobility of aluminum cans is the general trend in this manufacturing industry to increase production without additional capital investments in building new plants. The increased production demand is requiring can manufacturers to increase their line and printer speeds to produce 20 to 40 percent more cans per unit of time. For example, the maximum speed at which aluminum cans may be passed through a printing station typically is on the average of about 1150 cans per minute, whereas it is desired that such rate be increased to about 1400 to 1500 cans per minute or even higher.

However, thoroughly cleaned aluminum cans by either acid or alkaline cleaner are, in general, characterized by high surface roughness and thus have a high coefficient of static friction. This property hinders the flow of cans through single filers and printers when attempting to increase their line speed. As a result, printer misfeeding problems, frequent jammings, down time, and loss of production occur in addition to high rates of can spoilage.

Another consideration in modifying the surface properties of aluminum cans is the concern that such may interfere with or adversely affect the ability of the can to be printed when passed to a printing or labeling sta-

tion. For example, after cleaning the cans, labels may be printed on their outside surface as well as lacquers may be sprayed on their inside surface. In such case, the adhesion of the paints and lacquers is of major concern.

5 In addition, the current trend in the can manufacturing industry is directed toward using thinner gauges of aluminum metal stock. The down-gauging of aluminum can metal stock has caused a production problem in that, after washing, the cans require a lower drying 10 oven temperature in order to pass the column strength pressure quality control test. However, lowering the drying oven temperature resulted in the cans not being dry enough when they reached the printing station, and caused label ink smears and a higher rate of can rejects.

15      Thus, it would be desirable to provide a means of improving the mobility of aluminum cans through filers and printers to increase production, reduce line jamming, minimize down time, reduce can spoilage, improve ink laydown, and enable lowering the drying oven temperature of washed cans. Accordingly, it is an object of this invention to provide such means of improving the mobility of aluminum cans and to overcome the afore-noted problems.

### 3. Description of the Invention

25 Other than in the operating examples, or where otherwise indicated, all numbers expressing quantities of ingredients or reaction conditions used herein are to be understood as modified in all instances by the term "about".

30 about . In accordance with this invention, it has been found  
that a lubricant and surface conditioner applied to alu-  
minum cans after washing enhances their mobility and  
improves their water film drainage and evaporation  
characteristics as to enable lowering the temperature of  
35 a drying oven by from about 25° to about 100° F. with-  
out having any adverse effect on the label printing pro-  
cess. The lubricant and surface conditioner reduces the  
coefficient of static friction on the outside surface of the  
40 cans enabling a substantial increase in production line  
speeds, and in addition, provides a noticeable improve-  
ment in the rate of water film drainage and evaporation  
resulting in savings due to lower energy demands while  
meeting quality control requirements.

45 More particularly, in accordance with this invention, it has been found that application of a thin organic film to the outside surface of aluminum cans serves as a lubricant inducing thereto a lower coefficient of static friction, which consequently provides an improved 50 mobility to the cans, and also increases the rate at which the cans may be dried and still pass the quality control column strength pressure test. It has also been found that the improved mobility and drying rate of the cans depends on the thickness or amount of the organic film, 55 and on the chemical nature of the material applied to the cans.

The lubricant and surface conditioner for aluminum cans in accordance with this invention may be selected from water-soluble alkoxylated surfactants such as organic phosphate esters; alcohols; fatty acids including mono-, di-, tri-, and poly-acids; fatty acid derivatives such as salts, hydroxy acids, amides, esters, ethers and derivatives thereof; and mixtures thereof.

The lubricant and surface conditioner for aluminum cans in accordance with this invention preferably comprises a water-soluble derivative of a saturated fatty acid such as an ethoxylated stearic acid or an ethoxylated isostearic acid, or alkali metal salts thereof such as

polyoxyethylated stearate and polyoxyethylated isostearate. In addition, the lubricant and surface conditioner for aluminum cans may comprise a water-soluble alcohol having at least about 4 carbon atoms and may contain up to about 50 moles of ethylene oxide. Excellent results have been obtained when the alcohol comprises polyoxyethylated oleyl alcohol containing an average of about 20 moles of ethylene oxide per mole of alcohol.

Further, the lubricant and surface conditioner for aluminum cans in accordance with this invention may comprise a phosphate acid ester or preferably an ethoxylated alkyl alcohol phosphate ester. Such phosphate esters are commercially available under the tradename Gafac PE 510 from GAF Corporation, Wayne, N.J., and as Ethfac 136 and Ethfac 161 from Ethox Chemicals, Inc., Greenville, S.C. In general, the organic phosphate esters may comprise alkyl and aryl phosphate esters with and without ethoxylation.

The lubricant and surface conditioner for aluminum cans may be applied to the cans during their wash cycle, during one of their treatment cycles, during one of their water rinse cycles, or more preferably, during their final water rinse cycle. In addition, the lubricant and surface conditioner may be applied to the cans after their final water rinse cycle, i.e., prior to oven drying, or after oven drying, by fine mist application from water or another volatile non-inflammable solvent solution. It has been found that the lubricant and surface conditioner is capable of depositing on the aluminum surface of the cans to provide them with the desired characteristics. The lubricant and surface conditioner may be applied by spraying and reacts with the aluminum surface through chemisorption or physisorption to provide it with the desired film.

Generally, in the cleaning process of the cans, after the cans have been washed, they are typically exposed to an acidic water rinse. In accordance with this invention the cans may thereafter be treated with a lubricant and surface conditioner comprising an anionic surfactant such as a phosphate acid ester. In such case, the pH of the treatment system is important and generally should be acidic, that is between about 1 and about 6.5, preferably between about 2.5 and about 5. If the cans are not treated with the lubricant and surface conditioner of this invention after the acidic water rinse, the cans are exposed to a tap water rinse and then to a deionized water rinse. In such event, the deionized water rinse solution is prepared to contain the lubricant and surface conditioner of this invention which may comprise a nonionic surfactant selected from the aforementioned polyoxyethylated alcohols or polyoxylated fatty acids. After such treatment, the cans may be passed to an oven for drying prior to further processing.

The amount of lubricant and surface conditioner to be applied to the cans should be sufficient to reduce the coefficient of static friction on the outside surface of the cans to a value of about 1.5 or lower, and preferably to a value of about 1 or lower. Generally speaking, such amount should be on the order of from about 3 mg/m<sup>2</sup> to about 60 mg/m<sup>2</sup> of lubricant and surface conditioner to the outside surface of the cans.

For a fuller understanding of the invention, reference should be made to the following examples which are intended to be merely descriptive, illustrative, and not limiting as to the scope of the invention.

## EXAMPLE I

This example illustrates the amount of aluminum can lubricant and surface conditioner necessary to improve their free mobility through the tracks and printing stations of an industrial can manufacturing facility, and also shows that the lubricant and surface conditioner does not have an adverse effect on the adhesion of labels printed on the outside surface as well as of lacquers sprayed on the inside surface of the cans.

Uncleaned aluminum cans obtained from an industrial can manufacturer were washed clean with an alkaline cleaner available from the Parker + Amchem Division, Henkel Corporation, Madison Heights, Mich., employing that company's Ridoline ® 3060/306 process. The cans were washed in a laboratory miniwasher 35 processing 14 cans at a time. The cans were treated with different amounts of lubricant and surface conditioner in the final rinse stage of the washer and then 20 dried in an oven. The lubricant and surface conditioner comprised about a 10% active concentrate of polyoxyethylated isostearate, an ethoxylated nonionic surfactant, available under the tradename Ethox MI-14 from Ethox Chemicals, Inc., Greenville, S.C. The treated cans were 25 returned to the can manufacturer for line speed and printing quality evaluations. The printed cans were divided into two groups, each consisting of 4 to 6 cans. All were subjected for 20 minutes to one of the following adhesion test solutions:

30 Test Solution A; 1% Joy ® (a commercial liquid dishwashing detergent, Procter and Gamble Co.) solution in 3:1 deionized water:tap water at a temperature of 180° F.

35 Test Solution B; 1% Joy ® detergent solution in deionized water at a temperature of 212° F.

After removing the printed cans from the adhesion test solution, each can was cross-hatched using a sharp metal object to expose lines of aluminum which showed through the paint or lacquer, and tested for paint adhesion. 40 This test included applying Scotch (Scotch is a registered trademark of the 3M Company) transparent tape No. 610 firmly over the cross-hatched area and then drawing the tape back against itself with a rapid pulling motion such that the tape was pulled away from the cross-hatched area. The results of the test were 45 rated as follows: 10, perfect, when the tape did not peel any paint from the surface; 8, acceptable; and 0, total failure. The cans were visually examined for any print or lacquer pick-off signs.

50 In addition, the cans were evaluated for their coefficient of static friction using a laboratory static friction tester. This device measures the static friction associated with the surface characteristics of aluminum cans. This is done by using a ramp which is raised through an 55 arc of 90° by using a constant speed motor, a spool and a cable attached to the free swinging end of the ramp. A cradle attached to the bottom of the ramp is used to hold 2 cans in horizontal position approximately 0.5 inches apart with the domes facing the fixed end of the ramp. A third can is laid upon the 2 cans with the dome facing the free swinging end of the ramp, and the edges of all 3 cans are aligned so that they are even with each other.

60 As the ramp begins to move through its arc a timer is automatically actuated. When the ramp reaches the angle at which the third can slides freely from the 2 lower cans, a photoelectric switch shuts off the timer. It is this time, recorded in seconds, which is commonly 65

referred to as "slip time". The coefficient of static friction is equal to the tangent of the angle swept by the ramp at the time the can begins to move.

The average values for the adhesion test and coefficient of static friction evaluation results are summarized in Table 1 which follows:

TABLE 1

| Test No. | Lubricant and Surface Conditioner | Adhesion Evaluation |      |     | Coefficient of Static Friction |
|----------|-----------------------------------|---------------------|------|-----|--------------------------------|
|          |                                   | Test Solution       | OSW  | ISW |                                |
| 1        | Control (no treatment)            | —                   | —    | —   | 1.42                           |
| 2        | 0.1                               | B                   | 10   | 10  | 0.94                           |
| 3        | 0.25                              | A                   | 10   | 10  | —                              |
| 4        | 0.5                               | B                   | 9.5* | 10  | 0.80                           |
| 5        | 0.75                              | A                   | 10   | 10  | 0.63                           |
| 6        | 1.0                               | B                   | 10   | 10  | 0.64                           |
| 7        | 2.0                               | A                   | 10   | 10  | 0.56                           |
| 8        | 5.0                               | B                   | 10   | 10  | 0.55                           |
| 9        | 10.0                              | A                   | 9.8* | 10  | 0.56                           |

\*Little pick-off was visually noticed on the outside walls, mainly at the contact marks. In Table 1, OSW stands for outside sidewall, ISW stands for inside sidewall, and ID stands for inside dome.

In brief, it was found that the lubricant and surface conditioner concentrate as applied to the cleaned aluminum cans provided improved free mobility to the cans even at very low use concentrations, and it had no adverse effect on either adhesion of label print or internal lacquer tested even at 20 to 100 times the required use concentration to reduce the coefficient of static friction of the cans.

#### EXAMPLE II

This example illustrates the use of the aluminum can lubricant and surface conditioner of Example I in an industrial can manufacturing facility when passing cans through a printing station at the rate of 1260 cans per minute.

Aluminum can production was washed with an acidic cleaner (Ridoline ® 125 CO, available from the Parker + Amchem Division, Henkel Corporation, Madison Heights, Mich.), and then treated with a non-chromate conversion coating (Alodine ® 404). The aluminum can production was then tested for "slip" and the exterior of the cans were found to have a static coefficient of friction of about 1.63. During processing of these cans through a printer station, the cans could be run through the printer station at the rate of 1150 to 1200 cans per minute without excessive "trips", i.e., improperly loaded can events. In such case, the cans are not properly loaded on the mandrel where they are printed. Each "trip" causes a loss of cans which have to be discarded because they are not acceptable for final stage processing.

About 1 ml/liter of aluminum can lubricant and surface conditioner was added to the deionized rinse water system of the can washer which provided a reduction of the static coefficient of friction on the exterior of the cans to a value of 1.46 or a reduction of about 11 percent from their original value. After passing the cans through the printer, it was found that the adhesion of both the interior and exterior coatings were unaffected by the lubricant and surface conditioner. In addition, the printer speed could be increased to its mechanical

limit of 1250 to 1260 cans per minute without new problems.

In similar fashion, by increasing the concentration of the aluminum can lubricant and surface conditioner to 5 the deionized rinse water system, it was possible to reduce the coefficient of static friction of the cans by 20 percent without adversely affecting the adhesion of the interior and exterior coatings of the cans. Further, it was possible to maintain the printer speed continuously 10 at 1250 cans per minute for a 24 hour test period.

#### EXAMPLE III

This example illustrates the use of other materials as the basic component for the aluminum can lubricant and 15 surface conditioner.

Aluminum cans were cleaned with an alkaline cleaner solution having a pH of about 12 at about 105° F. for about 35 seconds. The cans were rinsed, and then treated with three different lubricant and surface conditioners comprising various phosphate ester solutions. 20 Phosphate ester solution 1 comprised a phosphate acid ester (available under the tradename Gafac ® PE 510 from GAF Corporation, Wayne, N.J.) at a concentration of 0.5 g/l. Phosphate ester solution 2 comprised an ethoxylated alkyl alcohol phosphate ester (available under the tradename Ethfac ® 161 from Ethox Chemicals, Inc., Greenville, S.C.) at a concentration of 0.5 g/l. 25 Phosphate ester solution 3 comprised an ethoxylated alkyl alcohol phosphate ester (available under the tradename Ethfac ® 136 from Ethox Chemicals, Inc., Greenville, S.C.) at a concentration of 1.5 g/l.

The mobility of the cans in terms of coefficient of static friction was evaluated and found to be as follows:

35

|    | Phosphate ester solution | pH  | Coefficient of static friction |
|----|--------------------------|-----|--------------------------------|
| 1  | 1                        | 3.6 | 0.47                           |
| 2  | 2                        | 3.3 | 0.63                           |
| 3  | 3                        | 2.6 | 0.77                           |
| 40 | None                     | —   | 1.63                           |

The aforementioned phosphate ester solutions all provided an acceptable mobility to aluminum cans, but 45 the cans were completely covered with "water-break". It is desired that the cans be free of water-breaks, i.e., have a thin, continuous film of water thereon, because otherwise they contain large water droplets, and the water film is non-uniform and discontinuous. To determine whether such is detrimental to printing of the cans, 50 they were evaluated for adhesion. That is, the decorated cans were cut open and boiled in a 1% liquid dishwashing detergent solution (Joy ®) comprising 3:1 deionized water:tap water for ten minutes. The cans 55 were then rinsed in deionized water and dried. As in Example I, eight cross-hatched scribe lines were cut into the coating of the cans on the inside and outside sidewalls and the inside dome. The scribe lines were taped over, and then the tape was snapped off. The cans were rated for adhesion values. The average value results are summarized in Table 2.

#### TABLE 2

| Phosphate ester Solution | Adhesion Rating |     |     |
|--------------------------|-----------------|-----|-----|
|                          | OSW             | ISW | ID  |
| control                  | 10              | 10  | 10  |
| 1                        | 9.8             | 6.8 | 1.0 |
| 2                        | 9.8             | 10  | 10  |

TABLE 2-continued

| Phosphate ester<br>Solution | Adhesion Rating |     |    |
|-----------------------------|-----------------|-----|----|
|                             | OSW             | ISW | ID |
| 3                           | 10              | 10  | 10 |

In Table 2, OSW stands for outside sidewall, ISW stands for inside sidewall, and ID stands for inside dome.

For the control, it was observed that there was no pick-off (loss of coating adhesion) on either the outside sidewall, the inside sidewall or the inside dome of the cans.

For phosphate ester solution 1, it was observed that there was almost no pick-off on the outside sidewall, substantial pick-off on the inside sidewall, and complete failure on the inside dome of the cans.

For phosphate ester solution 2, it was observed that there was almost no pick-off on the outside sidewall, and no pick-off on the inside sidewall and no pick-off on the inside dome of the cans.

For phosphate ester solution 3, it was observed that there was no pick-off on the outside sidewall, the inside sidewall, and the inside dome of the cans.

#### EXAMPLE IV

This example illustrates the effect of the lubricant and surface conditioner of this invention on the water draining characteristics of aluminum cans treated therewith.

Aluminum cans were cleaned with acidic cleaner (Ridoline ® 125 CO followed by Alodine ® 404 treatment or Ridoline ® 125 CO only) or with an alkaline cleaner solution (Ridoline ® 3060/306 process), all the products being available from the Parker + Amchem Division, Henkel Corporation, Madison Heights, Mich., and then rinsed with deionized water containing about 0.3% by weight of the lubricant and surface conditioner of this invention. After allowing the thus-rinsed cans to drain for up to 30 seconds, the amount of water remaining on each can was determined. The same test was conducted without the use of the lubricant and surface conditioner. The results are summarized in Table 3.

TABLE 3

| Drain<br>Time<br>(sec) | Water Remaining<br>(g/can) |                  |
|------------------------|----------------------------|------------------|
|                        | DI Water                   | 0.3% Conditioner |
| 6                      | 2.4-3.0                    | nd               |
| 12                     | 2.1-3.5                    | 2.8              |
| 18                     | 2.2-3.5                    | 2.3              |
| 30                     | 1.8-3.4                    | 2.3              |

It was found that the presence of the lubricant and surface conditioner caused the water to drain more uniformly from the cans, and that the cans remain "water-break" free for a longer time.

#### EXAMPLE V

This example illustrates the effect of the oven dryoff temperature on the sidewall strength of aluminum cans. This test is a quality control compression test which determines the column strength of the cans by measuring the pressure at which they buckle. The results are summarized in Table 4.

TABLE 4

|   | OVEN<br>TEMPERATURE<br>(°F.) | COLUMN<br>STRENGTH<br>(PSI) |
|---|------------------------------|-----------------------------|
| 5 | 440                          | 86.25                       |
|   | 400                          | 87.75                       |
|   | 380                          | 88.25                       |
|   | 360                          | 89.25                       |

It can be seen from Table 4 that at an oven drying temperature of 380° F., a 2 psi increase was obtained in the column strength test compared to the value obtained at 440° F. oven temperature.

The higher column strength test results are preferred and required because the thin walls of the finished cans must withstand the pressure exerted from within after they are filled with a carbonated solution. Otherwise, cans having weak sidewalls will swell and deform or may easily rupture or even explode. It was found that the faster water film drainage resulting from the presence therein of the lubricant and surface conditioner composition of this invention makes it possible to lower the temperature of the drying ovens and in turn obtain higher column strength results. More specifically, in order to obtain adequate drying of the rinsed cans, the cans are allowed to drain briefly before entry into the drying ovens. The time that the cans reside in the drying ovens is typically between 2 and 3 minutes, dependent to some extent on the line speed, oven length, and oven temperature. In order to obtain adequate drying of the cans in this time-frame, the oven temperature is typically about 440° F. However, in a series of tests wherein the rinse water contained about 0.3% by weight of the lubricant and surface conditioner of this invention, it was found that satisfactory drying of the cans could be obtained wherein the oven temperature was lowered to 400° F., and then to 370° F., and dry cans were still obtained.

I claim:

1. A liquid lubricant and surface conditioner composition for application to at least one exterior surface of a cleaned aluminum can to improve the mobility of the can when conveyed, said composition consisting essentially of a solution of water and water-soluble ethoxylated organic material selected from the group consisting of ethoxylated fatty acids, salts of ethoxylated fatty acids, and mixtures thereof, said liquid lubricant and surface conditioner composition having a pH of between about 1 and about 6.5 and forming a film on the can surface when applied thereto and dried, thereby reducing the coefficient of static friction of said surface.

2. A composition according to claim 1 wherein the pH is between about 2.5 and about 5.

3. A composition according to claim 1 wherein in the water soluble organic material is selected from the group consisting of ethoxylated stearic and isostearic acids, salts thereof, and mixtures thereof.

4. A composition according to claim 3 wherein the fatty acid is stearic acid or isostearic acid.

5. A composition according to claim 3 wherein said water is deionized water.

6. A composition according to claim 2 wherein said water is deionized water.

7. A composition according to claim 1 wherein said water is deionized water.

8. An aluminum can, at least one exterior surface of which is coated with a film formed from water-soluble

ethoxylated organic material selected from the group consisting of ethoxylated fatty acids, salts of ethoxylated fatty acids, ethoxylated alcohols having at least 4 carbon atoms and containing up to about 20 moles of condensed ethylene oxide per mole of alcohol, ethoxylated alkyl alcohol phosphate esters, and mixtures thereof, the amount of film on said surface being sufficient to reduce the coefficient of static friction thereof, thereby improving the mobility of the can when conveyed.

9. An aluminum can according to claim 8 wherein the coated surface has a coefficient of static friction of about 1.5 or below.

10. An aluminum can according to claim 9 wherein the surface is coated with from about 3 to about 60 15 mg/m<sup>2</sup> of said film.

11. A process of reducing the coefficient of static friction on at least one exterior surface of a cleaned aluminum can thereby increasing the mobility of the can when conveyed comprising applying to said surface a liquid lubricant and surface conditioner composition consisting essentially of a solution of water and water-soluble ethoxylated organic material selected from the group consisting of ethoxylated fatty acids, salts of 20 ethoxylated fatty acids, ethoxylated alcohols having at least 4 carbon atoms and containing up to about 20 moles of condensed ethylene oxide per mole of alcohol, ethoxylated alkyl alcohol phosphate esters, and mixtures thereof, said liquid lubricant and surface conditioner composition having a pH of between about 1 and 25 about 6.5; and drying said surface to form thereon a film which reduces the coefficient of static friction of said surface.

12. A process according to claim 11 wherein the film coated surface of the can is subsequently printed, lacquered, or both without a substantial reduction in the adherence of the printing or lacquer to the surface. 35

13. A process comprising the steps of cleaning an aluminum can with an aqueous acidic or alkaline cleaning solution, drying the cleaned can, and subsequently 40 conveying the cleaned and dried can via automatic conveying equipment to a location where it is lacquered or decorated by printing or both, wherein the improvement comprises contacting at least one exterior surface of said aluminum can, prior to the last drying of said exterior surface before automatic conveying, with a lubricant and surface conditioner composition, thereby forming a film on the can surface to provide the surface of the can after drying with a coefficient of static friction that is not more than 1.5 and that is less than would be obtained on a can surface of the same type without such film coating.

14. A process according to claim 13, wherein said lubricant and surface conditioner composition is an aqueous solution comprising dissolved organic material 45 selected from the group consisting of ethoxylated phos-

phate esters; ethoxylated alcohols; ethoxylated fatty acids; ethoxylated hydroxy substituted fatty acids; salts, amides, ethers, and esters of ethoxylated fatty acids and of ethoxylated hydroxy substituted fatty acids; and mixtures thereof.

15. A process according to claim 14, wherein said lubricant and surface conditioner composition consists essentially of a solution of water and dissolved organic material selected from the group consisting of ethoxylated phosphate esters; ethoxylated alcohols; ethoxylated fatty acids; ethoxylated hydroxy substituted fatty acids; salts, amides, ethers, and esters of ethoxylated fatty acids and of ethoxylated hydroxy substituted fatty acids; and mixtures thereof.

16. A process according to claim 15 wherein the lubricant and surface conditioner composition has a pH between about 1 and about 6.5 and the dissolved organic material is selected from the group consisting of ethoxylated fatty acids, salts of ethoxylated fatty acids, ethoxylated alcohols having at least 4 carbon atoms and containing up to about 20 moles of condensed ethylene oxide per mole of alcohol, ethoxylated alkyl alcohol phosphate esters, and mixtures thereof.

17. A process according to claim 16 wherein the water-soluble ethoxylated organic material is stearic acid, isostearic acid, an alkali metal salt of stearic acid, an alkali metal salt of isostearic acid, or mixtures thereof.

18. A process according to claim 13 comprising at least one additional step selected from the group consisting of:

- (A) decorating by printing at least a part of the coated surface so as to obtain a dried printing having an adhesion to the can not significantly less than obtained on the same, but uncoated, surface;
- (B) lacquering at least a part of the coated surface so as to obtain a dried lacquer coat having an adhesion to the can not significantly less than obtained on the same, but uncoated, surface; and
- (C) a combination of steps (A) and (B) being applied to separate portions of the coated surface.

19. A process according to claim 18 wherein the lubricant and surface conditioner composition has a pH between about 1 and about 6.5 and consists essentially of a solution of water and water-soluble ethoxylated organic material selected from the group consisting of ethoxylated fatty acids, salts of ethoxylated fatty acids, ethoxylated alcohols having at least 4 carbon atoms and containing up to about 20 moles of condensed ethylene oxide per mole of alcohol, ethoxylated alkyl alcohol phosphate esters, and mixtures thereof.

20. A process according to claim 19 wherein the water-soluble organic material is stearic acid, isostearic acid, an alkali metal salt of stearic acid, an alkali metal salt of isostearic acid, or mixtures thereof.

\* \* \* \* \*